



US006000863A

# United States Patent [19]

[19]

Clough et al.

[11] Patent Number: 6,000,863

[45] Date of Patent: Dec. 14, 1999

- [54] **PHOTOGRAPHIC PROCESSING METHOD**

[75] Inventors: **Arthur H. Clough**, Hardwick; **Michael G. Dowling**, Boxford; **David R. Gilda**, Watertown, all of Mass.

[73] Assignee: **Polaroid Corporation**, Cambridge, Mass.

[21] Appl. No.: **09/038,223**

## Related U.S. Application Data

- [60] Provisional application No. 60/040,388, Mar. 11, 1997.  
[51] **Int. Cl.**<sup>6</sup> ..... **G03D 5/00**; G03D 5/06  
[52] **U.S. Cl.** ..... **396/604**; 396/606; 206/455  
[58] **Field of Search** ..... 396/33, 575, 604,  
396/606, 623, 647; 355/27-29, 406; 206/455

## References Cited

## U.S. PATENT DOCUMENTS

- |           |         |               |       |         |
|-----------|---------|---------------|-------|---------|
| 2,558,857 | 7/1951  | Land          | ..... | 396/33  |
| 2,848,931 | 8/1958  | Troidl        | ..... | 396/575 |
| 3,345,165 | 10/1967 | Land          | ..... | 430/404 |
| 3,416,921 | 12/1968 | Coenen        | ..... | 430/206 |
| 3,576,632 | 4/1971  | Bornemisza    | ..... | 430/404 |
| 3,615,482 | 10/1971 | Cronig        | ..... | 430/456 |
| 3,647,464 | 3/1972  | Smith         | ..... | 430/232 |
| 3,680,462 | 8/1972  | Cronig        | ..... | 396/606 |
| 3,681,254 | 8/1972  | Becker        | ..... | 430/404 |
| 3,689,272 | 9/1972  | Schwan et al. | ..... | 430/206 |

- |           |         |                          |         |
|-----------|---------|--------------------------|---------|
| 3,816,136 | 6/1974  | Goffe et al. ....        | 430/405 |
| 3,826,653 | 7/1974  | Jacobs et al. ....       | 430/206 |
| 3,907,563 | 9/1975  | Land ....                | 430/206 |
| 3,930,859 | 1/1976  | Corrigan ....            | 430/404 |
| 4,452,523 | 6/1984  | Douglas ....             | 396/33  |
| 4,605,608 | 8/1986  | Bullitt ....             | 430/206 |
| 4,690,884 | 9/1987  | DeBruyn, Jr. et al. .... | 430/206 |
| 5,200,295 | 4/1993  | Vermeulen et al. ....    | 430/206 |
| 5,229,246 | 7/1993  | Shibata et al. ....      | 430/217 |
| 5,440,366 | 8/1995  | Reiss et al. ....        | 396/33  |
| 5,478,703 | 12/1995 | Simons ....              | 430/383 |

## FOREIGN PATENT DOCUMENTS

0 800 114 A2 10/1997 European Pat. Off. .

*Primary Examiner*—D. Rutledge  
*Attorney, Agent, or Firm*—Gaetano D. Maccarone

## ABSTRACT

A method for photographic processing of an exposed photosensitive film wherein a plurality of photographic processing elements comprising a carrier layer and a photographic processing layer containing photographic processing material are brought into contact, consecutively, with the exposed photosensitive film whereby a visible image is formed in the film. Each photographic processing element is initially brought into contact with the photosensitive film with the application of pressure and the processing element and the film are allowed to remain in contact with each other for a required period of time, during which at least one, and preferably a plurality of, additional pressure applications are carried out.

## 17 Claims, 20 Drawing Sheets





FIG. 1B



FIG. 1C



FIG. 1D





## FIG. 1E





## FIG. 1G



FIG.2

**FIG. 3**



FIG. 5



FIG. 4A



FIG. 4C



FIG. 4B



FIG. 6C



**FIG. 6D**



FIG. 6A



FIG. 6B



FIG. 7C



FIG. 7B



FIG. 7A



FIG. 8C



FIG. 8B



FIG. 8A



FIG. 9A

FIG. 9B

FIG. 9C



FIG. 10D



FIG. 9D



**FIG. 10A**



**FIG. 10B**



FIG. 10C



FIG. 11

**FIG. 12**



**FIG. 13****FIG. 14**

**PHOTOGRAPHIC PROCESSING METHOD****REFERENCE TO RELATED APPLICATIONS**

This application claims the benefit of prior copending provisional application serial No. 60/040,388 filed Mar. 11, 1997.

**BACKGROUND OF THE INVENTION**

The invention is directed generally to a photographic processing method wherein an image is formed in an exposed photosensitive film and, more particularly, to such a method which utilizes photographic processing elements comprising a carrier layer and a photographic processing layer containing photographic processing materials.

Generally, it is known in the art to carry out photographic processing of an exposed photosensitive film with photographic processing elements which comprise a carrier layer and a photographic processing layer which contains photographic processing materials. U.S. Pat. No. 2,558,857 to

Land teaches bringing a sheet material having a viscous coating comprising a liquid composition including a developer and a silver halide solvent into contact with an exposed photosensitive layer to develop a latent image in the photosensitive layer and thereby form a visible image. A photographic processing method of this type is generally referred to in the art as "dry" since the photographic processing chemicals are included in a layer of the photographic processing element and the photographic processing elements take the place of the photographic processing solution baths utilized in conventional "wet" photographic processing methods.

The prior art also describes materials which may be used in the dry photographic processing techniques. U.S. Pat. No. 3,615,482 to Cronig teaches gelable photoprocessing solutions which comprise a photoprocessing solution and an amount of gel-forming carrageenan or furcellaran sufficient to cause gelation of the solutions. The gelled compositions are taught as being useful to develop, bleach, fix, wash, etc. exposed photographic films. U.S. Pat. No. 3,680,462 to Cronig teaches a photographic processing apparatus which utilizes gelled photographic processing compositions.

Variations of photographic processing using dry photographic processing elements have been described in the art. In one technique a single processing element is brought into contact with the photosensitive film to carry out photographic development. U.S. Pat. No. 5,440,366 to Reiss and Cocco teaches a photographic processing system and method wherein individual dry photographic processing elements are sequentially wrapped onto a single processing spool. One embodiment utilizes a processing spool which houses all the photosensitive processing sections carried on a single carrier layer such as, for example, a first processing section which contains a photographic developer, a second processing section which contains bleaching and fixing chemicals and a third processing section which contains washing and stabilizing chemicals. An exposed photosensitive film, which is housed in a separate cartridge is extracted from the cartridge and the first processing section is brought into contact with the film for a predetermined period of time following which the first processing section is separated from the film and the second processing section is brought into contact with the film for a requisite period of time. Subsequently, the second processing section and the film are separated from each other and the third processing section is brought into contact with the film for a requisite period of time. After the third processing section and the film are

separated from each other the photographic processing is complete and a visible image is formed in the film.

While there has been interest in carrying out photographic processing of exposed photosensitive film with dry processing elements, the systems and methods described in the prior art have not been entirely satisfactory insofar as providing the desired results. Accordingly, there is a continuing need for novel and improved systems and methods for forming images in exposed photosensitive films using dry photographic processing materials.

It is therefore an object of this invention to provide a novel photographic processing method.

It is another object to provide a photographic processing method wherein an exposed photosensitive film is processed with a plurality of dry photographic processing elements.

It is a further object of the invention to provide a photographic processing method wherein an exposed photosensitive film is processed with a plurality of separate dry photographic processing elements.

**SUMMARY OF THE INVENTION**

These and other objects and advantages are accomplished in accordance with the invention by providing a method for photographic processing of an exposed photosensitive film wherein a plurality of photographic processing elements, provided as individual sections of a single photoprocessing element or as separate photoprocessing elements, and each comprising a layer of a carrier material and a photographic processing layer containing photographic processing material are brought into contact, consecutively, with the exposed photosensitive film whereby a visible image is formed in the film. Each photographic processing element is initially brought into contact with the photosensitive film with the application of pressure and the processing element and the film are allowed to remain in contact with each other for the photographically required period of time, during which at least one, and preferably a plurality of additional pressure applications are carried out. It has been found that the application of pressure during the period the photosensitive film and the photographic processing element are in contact with each other provides significant improvement in the visible image which is formed in the photosensitive film after photographic processing is complete. The images developed according to the method of the invention exhibit significantly improved uniformity of development, i.e., significant reduction of the numbers, and extent, of visual defects which are areas of poor or substantially no development. It is thought that the method of the invention, by applying pressure when the photosensitive film and the photoprocessing elements are initially brought together and applying pressure at least one additional time when the respective members are in contact with one another, provides a more uniform supply of photoprocessing chemicals to the film thus resulting in more uniform development.

The method of the invention can be carried out with any exposed silver halide photosensitive films which are designed to form multicolor images including those which provide a negative or a positive image. In a preferred embodiment, the method is carried out with an exposed photosensitive film which has at least two, and preferably three or more, silver halide emulsions which have been sensitized to different regions of the spectrum.

The photographic processing method of the invention utilizes at least two photographic processing elements such as, for example, a developer element and a fixing element or a developer element and a bleaching and fixing ("blix")

element. In a preferred embodiment four photographic processing elements are employed, i.e., a developer element, a bleaching element, a fixing element and a washing element. The individual photographic processing elements can have separate carrier layers in which case the elements are typically provided in separate spools or each of the photographic processing elements can be provided as separate sections on a single carrier layer and the element is provided in one spool.

The application of pressure in accordance with the photographic processing method of the invention may be carried out with any of many pressure-applying implements including by means of rollers, brushes, a knife-edge, a press, etc. In a preferred embodiment pressure is applied by one or more rollers as will be described in more detail below herein. The method can be carried out in conjunction with various types of apparatus.

#### BRIEF DESCRIPTION OF THE DRAWINGS

The aforementioned aspects and other features of the invention are described in detail in conjunction with the accompanying drawings in which the same reference numerals are used throughout for denoting corresponding elements and wherein:

FIGS. 1A-1G illustrate a first embodiment of a processing system, which can be used to carry out the method of the invention, at various stages of operation;

FIG. 2 is a perspective exploded view of one type of spool caddy for use with the processing system of FIGS. 1A-1G;

FIG. 3 is a perspective view of the assembled spool caddy of FIG. 2 with single processing spool installed;

FIG. 4A is a top view of the body of the spool caddy of FIG. 2;

FIG. 4B is a bottom view of the body of the spool caddy of FIG. 2;

FIG. 4C is a top view of the body of the spool caddy of FIG. 2 having both processing spools and a photographic roll film cartridge supported thereon;

FIG. 5 illustrates an alternative snap plate for use with the spool caddy of FIG. 2;

FIG. 6A illustrates an alternative binding lever for use with the spool caddy of FIG. 2 in conjunction with the snap plate of FIG. 5;

FIG. 6B is a magnified top view of a centrally located section of the snap plate of FIG. 5;

FIG. 6C is a schematical cross-sectional view of the binding lever of FIG. 6A in the unlocked position as installed in the spool caddy of FIG. 2;

FIG. 6D is a schematical cross-sectional view of the binding lever of FIG. 6A in the locked position as installed in the spool caddy of FIG. 2;

FIG. 7A is a perspective view of a photographic film cartridge to be processed by the processing system of FIGS. 1A-1G;

FIG. 7B is a side view of the photographic film cartridge of FIG. 7A;

FIG. 7C is a top view of the photographic film cartridge of FIG. 7A;

FIG. 8A is a perspective view of a processing spool for use with the processing system of FIGS. 1A-1G;

FIG. 8B is a cross-sectional side cutout view of the processing spool of FIG. 8A;

FIG. 8C is a top view of the processing spool of FIG. 8A;

FIG. 9A is a cross-sectional side view of two adjacent spiral walls, without a braking mechanism, mounted on a turntable to form a channel through which a film cartridge or processing spool can travel during film processing;

FIG. 9B is a cross-sectional side view of two adjacent spiral walls, including a braking mechanism, mounted on a turntable to form a channel through which a film cartridge or processing spool can travel during film processing;

FIG. 9C is a cross-sectional side view of two adjacent spiral walls, including a braking mechanism, mounted on a turntable to form a channel through which a processing spool is traveling during film processing;

FIG. 9D is a cross-sectional side view of two adjacent spiral walls, including a braking mechanism, mounted on a turntable to form a channel through which a film cartridge is traveling during film processing;

FIG. 10A is a perspective view of a spool retrieval mechanism used in the processing system of FIGS. 1A-1G;

FIG. 10B is a top view of a spool retrieval mechanism used in the processing system of FIGS. 1A-1G;

FIG. 10C is a left side view of a spool retrieval mechanism used in the processing system of FIGS. 1A-1G;

FIG. 10D is an end view of a spool retrieval mechanism used in the processing system of FIGS. 1A-1G;

FIG. 11 is a perspective overview of the processing system of FIG. 1A;

FIG. 12 is a top view of a second embodiment of a processing system which can be used to carry out the method of the invention;

FIG. 13 is a side cross-sectional view of a portion of a turntable used in the processing system of FIG. 12; and

FIG. 14 is a side cross-sectional view of a portion of the turntable used in the processing system of FIG. 12 in cooperation with a turntable support and guiding structure.

#### DESCRIPTION OF THE PREFERRED EMBODIMENTS

As mentioned previously the method of the invention can be carried out to form a visible image in any exposed silver halide photosensitive film which is designed to form a multicolor image. The method is preferably utilized to carry out photographic processing of photosensitive films which are suitable for the well known C-41 color processing. Such photosensitive films include the conventional color films which include two, or preferably three or more, silver halide photosensitive emulsions which are sensitized to different regions of the spectrum. Another type of film which can be processed according to the method of the invention is a photosensitive film which typically includes only a single silver halide layer but also includes dye precursors that are converted to dyes in direct proportion to the intensity of the silver image whereby, in effect, two images develop simultaneously, i.e., the silver image and the multicolor image. During processing the silver image is removed leaving the desired color image. Such films are commercially available. For a discussion of such films see Shutterbug, F. E. Schultz and R. W. Hicks, June 1997, pages 166-178.

The photographic processing method of the invention will be described in detail in conjunction with the specific processing systems illustrated in the Figures. Referring now to FIG. 1A there is seen a photographic processing system 200 which utilizes a spool caddy 1 as disclosed in copending, commonly assigned provisional application serial No. 60/040,662 filed Mar. 11, 1997, for retaining and

The photographic processing method of the invention will be described in detail in conjunction with the specific processing systems illustrated in the Figures. Referring now to FIG. 1A there is seen a photographic processing system 200 which utilizes a spool caddy 1 as disclosed in copending, commonly assigned provisional application serial No. 60/040,662 filed Mar. 11, 1997, for retaining and

supporting a film cartridge and a plurality of processing spools; in the embodiment illustrated there are shown four processing spools, three of which contain a photographic processing element and the fourth of which contains a blotter material.

### THE SPOOL CADDY

FIG. 2 is a perspective exploded view of one type of spool caddy 1. The three major components of the spool caddy 1 are the body 10, the snap plate 40 and the binding lever 60. Each of the major components is preferably molded or otherwise made from a strong, inexpensive, lightweight material such as polystyrene or any other plastic. These components when assembled together form the spool caddy 1, shown with a single processing spool 80 in FIG. 3.

The body 10 acts as means, as shown in FIG. 4C, for detachably and supporting a number of processing spools 80, 90, 100 and 110 as well as the film cartridge 70, in isolation from one another. The body 10 includes a base 12, a plurality of arms 14 and a wedge shaped cavity 20 centered along the central longitudinal axis 16 of the spool caddy 1. The cavity 20 is indexed, notched or keyed in a lower section of the body by a rectangular notch 22. Moreover, a slot 24 for engaging a film leader 76 of the film cartridge 70 (see FIGS. 4C and 7A) extends from the cavity 20 as shown. The body 10 also includes a notch 18, as shown in FIG. 3, acting as a means for enabling positional alignment of the spool caddy 1 in relation to other components of a photographic processing system.

The snap plate 40, having a thickness "z", includes a centrally located cavity shaped opening 46 similar in shape to the cavity 20 of the body 10, as well as a slot 25 corresponding to the slot 24 of the body 10. The snap plate 40 functions as means for detachably retaining or holding both a plurality of processing spools, such as the processing spool 80 of FIG. 3, and the film cartridge 70 of FIG. 7A. The snap plate 40 may be clover shaped as shown in FIG. 2, or its shape could vary as shown by the snap plate 140 of FIG. 5, as long as it has the ability to detachably retain processing spools and film cartridges. The snap plates 40 and 140 are both capable of detachably holding five spools, although the snap plates could be designed in cooperation with the spool caddy 1 to retain more or less spools if desired. The snap plate 40 of FIG. 2 includes five identical leaf shaped sections 50 defining five identical spaces therebetween, each space having a cross-sectional distance "a" and a narrow region of distance "m" at the perimeter of the snap plate 40. Similarly, the snap plate 140 of FIG. 5 includes five claw shaped arms 45 each having a pair of claws 49 and 51 which also define five identical spaces therebetween each having the same cross-sectional distance "a" and "m", respectively. The snap plate 40 or 140 and the body 10 can be glued together, snapped together, screwed together, or otherwise held together by any known fastening means. The spool caddy 1 of FIG. 2 provides clearance holes 42 in the snap plate 40 and raised bosses 44 on the body 10 which allow the two parts to be joined together by ultrasonic staking to form the body/snap plate assembly. The snap plate 140 of FIG. 5 includes clearance holes 43 which would be aligned with appropriately positioned raised bosses (not shown) replacing the bosses 44 on the body 10.

The snap plate 140 also includes centrally located cutouts 130, 132 and 134 as illustrated in FIGS. 5 and 6B. The cutout 130 is an hour glass-shaped opening defined by distances  $y_1$ ,  $y_2$  and  $y_3$ , where  $y_1=y_3=y_4$ ,  $y_4 < y_1$  and  $y_4 > y_2$  (see also FIG. 6A). Cutout 134 is separated from the cutout

130 by a section 133, and cutout 132 is separated from the cutout 130 by a section 131.

The binding lever 60 is designed as a means for detachably retaining, in cooperation with the body 10, a film leader 76 of the film 71. First, the film leader 76 is inserted into the cavity 20 of the caddy body 10, then the binding lever 60 is inserted through the top of the body/snap plate assembly so that the spring 62 is aligned with, and snaps into, the notch 22. The diameter  $x_5$  of the head 64 of the binding lever 60 is large enough so that the head 64 can not pass into or through the cavity 20. Also, the force of the spring 62 pushes the spring 62 against the internal wall of the notch 22 to securely bind the lever 60 in the cavity 20. Hence, once the binding lever 60 is inserted into the cavity 20 it cannot be removed. After insertion of the binding lever 60, the head 64 and the indent 66 of the binding lever 60 will both protrude above the snap plate 40 as shown in FIG. 3 to act in cooperation as a handle for inserting and removing the spool caddy 1 from a processing system.

The binding lever 60 of FIG. 2 includes: a shaft 68 of diameter  $x_6$  and height  $x_1$ ; an indent 66 of length  $X_3$ ; a head 64 having a diameter  $x_5$  and a thickness  $X_4$ ; and a spring 62 of length  $X_7$  having a spring force which tends to extend the spring 62 away from the shaft 68 as shown. When a force is applied to the spring 62 to bring it nearly parallel with the longitudinal axis 16 of the shaft 68 (shown by dotted lines), the length  $X_7$  defines the distance from the bottom of the shaft 68 to the top end of the spring 62. The length  $X_7$  also corresponds to the length "k" of the notch 22 located adjacent to the lower portion of the cavity 20 in the caddy body 10.

The distance  $x_1$  of the shaft 68 of the binding lever 60 equates to the sum of the height "w" of the caddy body 10 and the width "z" of the snap plate 40 so that when the spool caddy 1 is completely assembled as shown in FIG. 3, the shaft head 64 and the indent 66 both protrude above the snap plate 40.

Once the spool caddy 1 is assembled as shown in FIG. 3, any movement of the binding lever 60 in a direction crossing the central longitudinal axis 16 of the spool caddy 1 is hampered by the force of the spring 62. Furthermore, any movement of the binding lever 60 in a direction parallel to the longitudinal axis 16 is hampered by both the head 64 and the physical engagement of the spring 62 within the notch 22.

When the user decides to process the film within a 35 mm film cartridge 70 using a spool caddy 1 having a snap plate 40 and a binding lever 60, he first feeds the film leader 76 into the slot 24 of the caddy body 10 and along the flat surface 125 of the cavity 20 (see FIGS. 3, 4B and 4C). Next, the binding lever 60 is inserted as described above so that the spring 62 snaps into the notch 22 and the film leader 76 becomes bound between the shaft 68 and the flat surface 125 in the cavity 20. The film cartridge 70 is then detachably secured onto the spool caddy 1 by snapping the core 72 of the film cartridge 70 into the clover leaf shaped snap plate 40. In order to release the film leader 76, the user laterally applies pressure to the head 64 of the binding lever 60 so that the shaft 68 moves slightly away from the flat surface 125.

A second type of binding lever 120 for use with the snap plate 140 of FIG. 5 is shown in side view in FIG. 6A. The binding lever 120 includes a shaft 128 having a cutout section 126. The shaft 128 has a diameter  $y_4$ , and further includes an annular rib 122 having a diameter greater than  $y_4$ . The binding lever 120 is designed to operate in cooperation with the cutout section 130 of the snap plate 140 (see

FIGS. 5 and 6B). The binding lever 120 is placed in an initial unlocked position as shown in FIG. 6C by inserting lever 120 through  $y_3$  of the cutout 130 and into the body/snap plate assembly from the top until the spring 62 snaps into place within the notch 22.

When the user decides to process the film within a 35 mm film cartridge 70 using a spool caddy 1 having a snap plate 140, first, the film leader 76 is fed into the slot 24 of the caddy body 10 and into engagement with the flat surface 125 in the cavity 20. Then, the binding lever 120 is inserted into the unlocked position of FIG. 5C so that the film leader 76 is loosely positioned in the cavity 20 between the flat surface 125 and the shaft 128. A lateral force is then applied to the head 124 of the binding lever 120 so that the binding lever 120 is shifted and snapped into the locked position shown in FIG. 6D, whereby the film leader 76 is securely fastened in the cavity 20 between the flat surface 125 and the shaft 128. When pushing the binding lever 120 into the locked position, the binding lever 120 passes from  $y_3$  (see FIG. 6B) through the region  $y_2$  of the cutout 130 and into the locked position of FIG. 5D corresponding to the region  $y_1$  of the cutout 130. When the binding lever 120 passes through the region  $y_2$  of the cutout 130, the sections 131 and 133 will slightly bend away from the cutout 130 and into the respective cutouts 132 and 134, thus momentarily expanding the distance  $y_2$  to allow passage of the binding lever shaft 128. After passage of the binding lever 60, the sections 131 and 133 resiliently return to their original positions. The resultant locked position of the binding lever 120 is illustrated in FIG. 6D whereby the annular rib 122 is bound upon the inner surface 125 of the cavity 20 with the film leader 76 secured therebetween (not shown). Once the film leader 76 is secured within the cavity 20, the film cartridge 70 can be detachably secured onto the spool caddy 1 by snapping the core 72 of the film cartridge 70 between two claws 49 and 51 of the snap plate 140.

The film leader 76 can be readily removed from the binding lever 120 by moving the binding lever 120 into its unlocked or release position. This is accomplished by pushing the head 124 of the binding lever 120 from  $y_1$  through  $y_2$  and into  $y_3$ , as viewed in FIG. 6B, whereby the film leader 76 is then loosely positioned between the annular rib 122 of the shaft 128 and the flat surface 125 to facilitate removal therefrom.

The processing spools 80, 90, 100 and 110 are each installed into the spool caddy 1 in the same manner in which processing spool 80 is shown to be installed in FIG. 3. Each processing spool as well as a standard 35 mm film cartridge 70 contains a hollow core 72 with dual drive tangs 74 recessed therein (see FIGS. 7C and 8C) for transferring rotational drive force from a source (such as the spool drive motor 270 in FIG. 10D) to the spool or cartridge through its respective core 72.

The structure and dimensions of each processing spool 80, 90, 100 and 110 are similar to that shown in FIGS. 8A, 8B and 8C. FIG. 7B illustrates a typical 35 mm film cartridge 70 having a height  $D_4$  and a diameter  $D_8$ . The cartridge 70 includes a core 72 having a diameter  $D_{10}$  and a height  $D_9$  which protrudes from the main body of the film cartridge 70. FIG. 8B illustrates a developer processing spool 80 having a height  $D_{13}$  and a diameter  $D_7$ . The spool 80 includes a core 72 having a diameter  $D_{12}$  and a height  $D_{11}$  which protrudes from the main body of the spool 80. The processing spool 80 also includes upper and lower flanges 73 and 75, respectively, each having a thickness  $D_2$ . FIG. 8B further illustrates a partially unwound spool 80 whereby the photographic developer element 82 has been unwound by a

distance  $D_1$  from the outer edges, i.e. the circumference, of the equal sized flanges 73 and 75. The various dimensions of the film cartridge 70 and the processing spool 80 are related as follows:  $D_{10}=D_{12}$ ;  $D_9=D_{11}$ ;  $D_4=D_{13}$ ;  $D_7>D_8$ ; and  $D_{13}=D_3+2D_2$ . If a film cartridge has less than 24 exposures, then  $D_7\geq D_8$ .

The photographic developer element comprises a carrier layer which may be any suitable material which is stable to the chemical developer materials and has sufficient mechanical strength to resist tearing during processing. Typical suitable carrier layer materials include polymeric materials such as polyethylene terephthalate, polystyrene and cellulose acetate, coated papers and the like. The carrier layer, which may be of any suitable thickness, is typically from about 1 to about 5 mils or more (0.025 mm to 0.125 mm). Thinner carrier layers are preferred because they are more responsive to the pressure applied in carrying out the method of the invention. The photographic developer element further comprises a photographic developer layer of an absorbent material for holding the photographic developer solution. Absorbent materials which are suitable for use in such photographic processing layers are known in the art. Typical suitable absorbent materials include gel-forming carrageenans and furcellaran such as are described in U.S. Pat. 3,615,482 and sulfonated poly(vinyl alcohol) derivatives such as are described in U.S. Pat. 3,647,464. The absorbent layer typically has a thickness of from about 6 to about 12 mils or more (0.15–0.3 mm); a preferred thickness is from about 8 to about 10 mils (0.2–0.25 mm). The photographic developer solutions, as well as the bleaching, fixing and washing solutions, referred to in this illustrative embodiment are well known in the art and do not require any detailed discussion here. The amount of photographic developer solution incorporated into the photographic developer layer varies with the particular type of photosensitive film being processed and the processing parameters employed. Routine scoping experiments can be used to determine the optimum concentration of active developer species and the ratio of other solution components (or any of the other processing solutions used) for any particular photosensitive film and processing system. For processing of a standard 35 mm color negative film with standard C-41 phenylenediamine developer, it is preferred to have a coverage of from about 250 to about 350 mg/ft<sup>2</sup> (2691 to 3667 mg/m<sup>2</sup>). A particularly preferred coverage of developer is from about 300 to about 325 mg/ft<sup>2</sup> (3229 to 3498 mg/m<sup>2</sup>). A preferred absorbent material for use in the photographic processing elements utilized in accordance with the invention comprises a mixture of iota-carrageenan and kappa-carrageenan. A particularly preferred composition comprises 10% by weight iota-carrageenan and 90% kappa-carrageenan. For a discussion of the characteristics and properties of various types of carrageenans see the Handbook of Water-Soluble Gums and Resins, Chapter 5 Carrageenan, Davidson, McGraw Hill Book Company, 1980.

The absorbent layers of the photoprocessing elements used in accordance with the method of the invention should be sufficiently stiff such that the material can withstand the application of pressure as practiced according to the method and sufficiently pliable in order to be able to transfer the processing chemicals effectively to the film. Typically, the absorbent layer should have a degree of stiffness ("gel strength") of from about 500 to about 4000 g/cm<sup>2</sup> or more. Preferably the absorbent layer has a gel strength of from about 1000 to about 2500 g/cm<sup>2</sup>; a particularly preferred gel strength range is from about 1000 to about 1500 g/cm<sup>2</sup>.

The spool caddy 1 is designed to accommodate any film cartridge such as a 35 mm film cartridge or processing spool

by snapping the core 72 through the appropriate narrow region "m" of the snap plates 40 or 140 and into the space having a cross-sectional distance "a" as shown in FIGS. 2 and 5, whereby  $a=D_{10}=D_{12}$  and  $m < a$ . Since the length and thickness of the webs within the processing spools may likely be greater than the length and thickness of the image carrying medium within the film cartridge 70, then the diameter  $D_7$  of the processing spools may likely be greater than the diameter  $D_8$  of a standard size 35 mm film cartridge. Thus, the spool caddy 1 is built to accommodate spools having various diameters. Moreover, the snap plates 40 and 140 are made of a flexible, resilient plastic which allows resilient spreading of the leaf sections 50 in the snap plate 40 and the claws 49 and 51 in the snap plate 140 during insertion or removal of the core 72 of a spool or cartridge. Once a processing spool or a film cartridge is snapped into place in the spool caddy 1 as shown in FIG. 3, it is held there until a force is applied to remove the core 72 through the gap "m". The force required for inserting or removing the core 72 from either snap plate 40 or 140 is adjustable by changing the material from which the snap plate 40 or 140 is made, changing the thickness "z" of the snap plate 40 or 140, or by adjusting the length and width of a channel 47 for each arm 45 of the snap plate 140.

Each processing spool contains a photographic processing element having a protruding leader which is fixedly attached to one arm 14 of the caddy body 10 as shown in FIG. 4C. For example, the photographic processing element 82 of spool 80 is shown to have a protruding leader 86 which is fixedly attached to one arm 14 at point 84. In the embodiment illustrated spool 80 contains a photographic developer element 82 which has an absorbent layer imbued with developing chemicals; spool 90 contains a photographic blix element (i.e. bleaching and fixing) which has an absorbent layer imbued with a combination of bleaching and fixing chemicals; spool 100 contains a photographic wash element 102 which has an absorbent layer imbued with a combination of washing and stabilizing agents; and spool 110 contains a blotter element which contains a dry non-woven material. The blotter material, of course, does not contain any photographic processing chemicals.

The assembled spool caddy 1 contains the body 10, the snap plate 40, the binding lever 60, and the preselected processing spools. The number and contents of the processing spools of a particular spool caddy can vary according to the needs for processing a particular roll of film. For instance, if separate bleaching and fixing steps are desired, then the blix spool 90 could be replaced by two separate spools, one containing a processing element which has an absorbent layer imbued with bleaching chemicals, and the other containing a processing element which has an absorbent layer imbued with fixing chemicals. The spool caddy 1 would then require six arms 14 and the snap plate 40 would require six leaf shaped sections 50.

Of course, processing spools with other processing capabilities could be added to the spool caddy 1 if desired. The number of arms 14 on the caddy body 10 and the number of leaf shaped sections 50 on the snap plate 40, or claws 45 on the snap plate 140, can change in accordance with the number of spools desired or required for film processing. Moreover, the arms 14 can take any desired shape as long as they provide both support for the various spools, and isolation of those spools from one another. Also, any snap plate design may be used that allows the snap plate to detachably hold each spool in place. Furthermore, the processing spools could be encased in hard shell cartridges, similar to 35 mm cartridges, so that a snap plate could detachably retain the

bodies of the hard shell processing cartridges, rather than the cores as described above.

A modified version of the above-described spool caddy 1 would house only the processing spools, i.e. the modified spool caddy 1 would not house the film cartridge 70. In this embodiment, the structural components of the spool caddy 1 which interact solely with the film 71 or the film cartridge 70 become unnecessary. In other words, the binding lever 60, the slot 24 and the cavity 20 would no longer be needed.

Other embodiments of a spool caddy which can be used with the inventive processing system are described in copending commonly assigned provisional patent application serial No. 60/040,662 filed Mar. 11, 1997. The functionality of the spool caddy 1, in cooperation with other elements of a photographic processing system 200 according to the present invention, is hereinafter described.

#### STRUCTURE OF A PHOTOGRAPHIC PROCESSING SYSTEM

The photographic processing system 200 shown in FIG. 1A includes a housing 206, a heating unit 201 mounted within the housing 206, a turntable 202 fastened to the housing 206, and an overhead support structure which may be a bridge or, as illustrated, a cantilever 204 mounted onto a base assembly 208 which is, in turn, mounted upon a surface 226 of the housing 206. The turntable 202 includes a spiral shaped rib or wall 220 having an internal side 224 and an external side 222 with a foam rubber strip 221 adhesively bonded thereto between points A and C of the spiral. The turntable 202 also includes a recessed circular area 205 for accommodating the spool caddy 1. The circular area 205 has a slightly larger radius than the radius of the spool caddy 1, whereby the circular area 205 is recessed below the turntable surface 226 and centered at a rotational axis 233 of the turntable 202. Additionally, a protrusion 230 extends from the recessed circular area 205 for cooperation with a keyed notch 18 of the spool caddy 1 in order to keep the spool caddy 1 in a fixed position in relation to the turntable 202. Other known keying arrangements can be utilized as described, for instance, in copending application Ser. No. 60/040,662.

The turntable 202, as well known in the art, can be powered by a belt (not shown) and a motor 250, which is wired to and controlled by a controller 260, e.g. a servo controller. The motor 250 could be designed with a slip gear or pulley (not shown) which will harmlessly spin when a torque limit is reached while moving a spool or cartridge along the channel 203. As another option, a current limited locked rotor drive system could be used whereby the motor locks when its torque exceeds some preset limit.

The cantilever 204 is supported at one end by the base assembly 208 and, without further support, extends above the wall 220 to the vicinity of the spool caddy 1 (see FIG. 1A). The cantilever 204, preferably constructed from a beam of  $\frac{3}{8}$  inch square cross-sectional steel or some other strong durable material, acts as a support and guide for the spool retrieval mechanism 216 which will move back and forth along the cantilever 204 in accordance with a predetermined timing sequence dictated by the controller 260.

The spool retrieval mechanism 216 is shown from a perspective view in FIG. 10A, from a top view in FIG. 10B, from a left side view in FIG. 10C, and from an end view while engaging a spool in FIG. 10D. Movement of the spool retrieval mechanism 216 along the channel 203 is directed by the cam follower rollers 266 which are mounted on the bottom of the rear support block 258 and which continu-

## 11

ously engage the top edge 207 of the wall 220 (see FIG. 9A) as the spool retrieval mechanism 216 moves back and forth along the cantilever 204. Together with the cantilever 204, the spool retrieval mechanism 216 forms a means for transporting and winding or unwinding a spool or cartridge along the channel 203. The spool retrieval mechanism 216 includes both a front support block 252 and a rear support block 258.

The front support block 252 of the spool retrieval mechanism 216 has therethrough both a threaded bore 254 and a smooth square bore 256. The square bore 256 accepts the cantilever 204 for supporting and guiding the mechanism 216, and the threaded bore 254 accepts a threaded screw 291 which is an extension of the shaft 289 of the screw drive motor 262. The screw drive motor shaft 289 passes through the bore 293 in the rear support block 258. Other components attached to the front block 252 include a spool rewind motor 270, a spindle retraction solenoid 268, and a linkage 255 connected to the front block 252 by a pair of pivotal connectors 283.

The rear support block 258 of the spool retrieval mechanism 216 has attached thereto: a spread roll solenoid 264 mounted to the block 258 by connectors 287; the screw drive motor 262; and a pair of cam follower rollers 266. The cam followers 266 are designed to extend below the rear support block 258 so that they engage and follow both the interior and exterior surfaces 224, 222 of the wall 220 along a section within a distance  $D_{18}$  (see FIG. 9B) of the top edge 207 of the wall 220.

The spread roll solenoid 264 has a shaft 261 which moves in and out of a bore 265 and which is pivotally connected to one end of an extender 257 by a pivotal connector 285. The other end of the extender 257 is pivotally connected to the linkage 255 by a pivotal connector 271. The linkage 255 is further pivotally connected to a spread roller support 253 by a pivotal connector 259. A cylindrical, rubber covered spreading roller 210, having a central longitudinal axis 275, is mounted along the axis 275 to the support 253, for instance, by pins 277 which can snap into indents (not shown) that are machined into each end 279 and 281 of the spread roller 210.

When the spread roll solenoid 264 is activated by the controller 260, the shaft 261 is retracted so that the spreading roller 210, through the component set 257, 255 and 253, is retracted and disengaged from the external side 222 of the wall 220 as shown in FIG. 10B. Specifically, when the shaft 261 retracts into the bore 265 of the solenoid 264, the extender 257 is also drawn towards the solenoid 264 so that the linkage 255 moves in the direction of the solenoid 264 along a circular path centered by the axis 267 (FIG. 10A) which is created by joining the connectors 283 together with a straight line. In this manner, the spread roller 210 also moves in the direction of the solenoid 264 so that the roller 210 moves away from the external surface 222 of the wall 220 to which the roller 210 was engaged.

When the solenoid 264 is deactivated, the force of the spring 263 returns the shaft 261 to its extended position so that, through the component set 257, 255 and 253, the spreading roller 210 becomes engaged with the external side 222 of the wall 220 as shown for instance in FIG. 1D. Specifically, when the shaft 261 extends out of the bore 265 of the solenoid 264, the extender 257 is moved away from the solenoid 264 along a radial path centered by the axis 267. In this manner, the spread roller 210 is radially moved away from the solenoid 264 until the roller 210 becomes engaged with the external surface 222 of the wall 200 using a

## 12

predetermined engagement force from the spring 263 (see FIG. 10A). Also when the solenoid 264 is deactivated, the pivotal movement of the spreading roller 210 and the support 253 about the pivotal connector 259 allows the roller 210 to accurately track the external surface 222 of the wall 220 through any irregularities so that the rubber cylindrical surface of the roller 210 remains in full contact with the external surface 222.

The front support block 252 can be moved in relation to the rear support block 258. The front and rear support blocks 252 and 258, respectively, are originally positioned adjacent to one another as shown in FIG. 10A, but the front support block 252 can be moved to an extended position as shown in FIG. 1C. The shaft 291 of the screw drive motor 262 engages with the threaded bore 254 of the front support block 252, thus enabling relative movement of the front support block 252 to the rear support block 258 upon activation of the screw drive motor 262.

With the front support block 252 in the extended position away from the rear support block 258, the screw drive motor 262 is activated in a reverse direction so that the front support block 252 will move towards the rear support block 258. In accordance with instructions from the controller 260, the screw drive motor 262 will function for a given time at a given rate in the reverse direction, causing the front support block 252 to move to a position adjacent to the rear support block 258.

When the front support block 252 is adjacent to the rear support block 258, the screw drive motor 262 can be activated in a forward direction to move the front support block 252 away from the rear support block 258. In accordance with instructions from the controller 260, the screw drive motor 262 will function for a given time at a given rate so that the front support block 252 will move a predetermined distance away from the rear support block 258. This distance will correspond with positioning the spindle 276 directly over the core 72 of a spool or cartridge housed in the spool caddy 1 (see FIG. 1C).

When the screw drive motor 262 is activated to position the front support block 252 over a spool or cartridge housed on the spool caddy 1, the intent is to secure the spool or cartridge so that it can be moved along the channel 203 of the spiral wall 220 to unwind a photographic processing element or film.

The spool rewind motor 270 has a shaft 274 which is inserted into and fixedly attached to a spool drive spindle 276 having a spindle head 278 connected at one end thereof. The spool rewind motor 270 is activated for rewinding a spool or cartridge. When the spool rewind motor 270 is deactivated, the shaft 274 and the spindle 276 rotate freely. The spindle 276 contains a flange 280 and a spindle bore 282 having bearings 295 in the front support block 258. The flange 280 regulates the movement of the spindle 276 through the bore 282, and also allows transmission of spring force from the spring 285 when the spindle 276 is lowered into the core 72 of a spool. The spindle assembly 286, which includes the motor 270, the shaft 274 and the spindle 276, is linked to the shaft 272 of the spindle retraction solenoid 268 via a linkage 284. When the solenoid 268 is activated, the shaft 272 is retracted into the bore 297 of the solenoid 268, causing the linkage 284 (as shown by dotted lines in FIG. 10C) to be pulled towards the solenoid 268 which, in turn, causes the spindle assembly 286 to move to an upper position whereby the spindle head 278 retracts into the bore 282. At this point, the front support block 252 can be moved (without the spindle head 278 striking the wall 220) to

position the spindle 276 directly above the core 72 of a spool or cartridge housed in the spool caddy 1 as shown in FIG. 1C. When the spindle retraction solenoid 268 is deactivated, the spring 285 causes the shaft 272 to be extended out of the solenoid 268 so that the spool assembly 286 is moved, via linkage 284, to a lower position, causing the spindle head 278 to engage the tangs 74 of the spool core 72 as shown in FIG. 10D. Once the spindle head 278 is engaged with the tangs 74 of the spool core 72, the screw drive motor 262 is activated in the reverse direction to draw the front support block 252 adjacent to the rear support block 258. Then, the spool or cartridge can be moved along the channel 203 by rotational movement of the turntable 202.

The above example describes but one embodiment of a device for moving a selected photographic processing spool, e.g., 80, to and from the spool caddy 1, and along the channel 203. An alternative spool retention and movement mechanism could be designed, as known by those skilled in the art, which would retain both the top and bottom ends of a photographic processing spool, e.g., spool 80. The spool core 72 located at the top end of the spool 80 could be retained as previously described (see FIG. 10D), and the bottom (i.e. opposite) end of the spool 80 could be retained by a mechanism (not shown) housed in the trench 223 of the turntable 202 (see FIGS. 12 and 13).

A preferred structure for guiding and supporting the turntable 202 on the housing 206 of the photographic processing system 200 includes triangularly located guide and support structures 225 (FIG. 12) which can be designed, for instance, to cooperate with the turntable 202 as shown in FIG. 14.

The photographic processing system 200 also requires a light-tight, cover 299 as shown in FIG. 11 so that when the cover is closed and the system 200 is activated, no light will enter the system. Furthermore, the heating unit 201 will heat and maintain the closed system 200 at the requisite processing temperature, e.g., about 103° F. throughout processing by insulating both the housing 206 and the cover 299 and regulating, by use of a thermostat (not shown), the temperature within the closed system 200.

#### OPERATION OF THE PHOTOGRAPHIC PROCESSING SYSTEM

The operation of the first embodiment of the photographic processing system 200 will now be described in view of FIGS. 1A-1G for processing a film cartridge which houses 36 exposures. A system user first inserts an exposed film cartridge 70 into the spool caddy 1 in the manner previously described, then mounts the spool caddy 1 into the keyed recessed circular area 205 of the turntable 202 as shown in FIG. 1A so that the central longitudinal axis 16 of the spool caddy 1 aligns with the rotational axis 233 of the turntable 202. Note that the spool caddy 1 is illustrated without a snap plate 40 or 140 in FIGS. 1A-1G for easier viewing of the underlying processing spools. Of course in actual operation, the spool caddy 1 would be completely assembled as shown, for instance, in FIG. 3.

The spool retrieval mechanism 216 is initially located along the cantilever 204 as shown in FIG. 1A. The spool caddy 1 and the turntable 202 are keyed together so that when the turntable 202 is rotated, both the turntable 202 and the spool caddy 1 will have the same angular rotation rate about the axis 233. After the spool caddy 1 is securely positioned upon the turntable 202 as shown, the light-tight cover 299 is then closed (see FIG. 11) and the system 200 is activated by use of a control panel (not shown) to begin

sequential operations described hereinafter under the control of the controller 260, such as a microprocessor.

Each spool or cartridge will be unwound along channel 203 as necessary for processing. A 12 exposure film cartridge will be unwound to point A, a 24 exposure film cartridge will be unwound to point B, and a 36 exposure cartridge will be unwound to point C. Each processing step will time out after an appropriate predetermined period of time. For instance, if the predetermined travel time of moving a spool or cartridge from the spool caddy 1 to point C is, say, 15 seconds, then each unwinding stage during the photographic processing of a film cartridge would last for 15 seconds. If the 12 exposure film cartridge reaches point A and is completely unwound after 5 seconds, then the motor 250 will continue to run for another 10 seconds until it times out. Alternatively, the time outs could vary depending upon the operator selection for processing different length films.

After the spool caddy 1 has been inserted and the system activated, the spindle retraction solenoid 268 is activated causing the spindle 276 of the spool retrieval mechanism 216 to retract into the spindle bore 282. The turntable 202 is rotated clockwise until the spool retrieval mechanism 216 is positioned in line with the blotter spool 110 as shown in FIG. 1B. At that point, the turntable 202 is momentarily halted and the screw drive motor 262 is activated in the forward direction to extend the front support block 252 of the spool retrieval mechanism 216 as previously discussed until it is positioned above the core 72 of the blotter spool 110 as shown in FIG. 1C. Then, the spindle retraction solenoid 268 is deactivated so that the head 278 of the spindle 276 drops into engagement with the tangs 74 of the blotter spool 110 in the same manner as illustrated in FIG. 10D where the spindle head 278 engages with the tangs 74 of a spool 80. After the spindle head 278 engages the tangs 74, the screw drive motor 262 is activated in the reverse direction until the front support block 252 is adjacent to the rear support block 258 and the blotter spool 110 is positioned in the channel 203. At this point in time, the spread roll solenoid 264 is deactivated, causing the spreading roller 210 to engage with the external side 222 of the wall 220 as previously discussed. Then, the turntable 202 is rotated counterclockwise until the blotter material 111 of the blotter spool 110 is completely unwound and located adjacent to the end stop 227 at position C along the spiral wall 220. The spreading roller 210, when engaged, rolls the blotter material 111 along the external surface 222 of the wall 220, resulting in an even spreading of the blotter material 111. It is now desirable to park the blotter spool 110 at point C as shown in FIG. 1D so that the spool retrieval mechanism 216 can retrieve other spools from the spool caddy 1. It should be noted here that the use of the non-woven blotter material, although a preferred embodiment, is optional. The blotter material serves to absorb any excess processing chemicals.

A braking mechanism or means for holding a spool or cartridge at a fixed position along the channel 203 is shown in FIGS. 9B, 9C and 9D. FIG. 9A is a cross-sectional side view of the channel 203 defined by the turntable 203 and two adjacent sections of the spiral wall 220 having a width  $D_6$ . The channel 203 has a width  $D_{13}$  and a height  $D_{14}$ . A brake pad 221 having a height  $D_5$  and a thickness  $D_{16}$  is adhesively bonded to the inner surface 224 of the wall 220 as shown in FIG. 9B. The brake pad 221, positioned a distance  $D_{17}$  from the bottom surface 236 of the channel 203 and a distance  $D_{15}$  from the top edge 207 of the wall 220, is preferably made of a resilient material such as foam rubber. FIG. 9C shows a processing spool 80 traveling through the channel 203 while engaging the brake pad 221. Specifically, the partially

unwound processing spool 80 first engages the brake pad 221 at point A on the processor 200 (see FIG. 1A), so that approximately one-third of the web is unwound from the spool 80 as viewed in FIG. 9C. Note that the brake pad 221 is adhesively bonded to the inner surface 224 of the wall 220 whereas the web 82 of the developer spool 80 is being unwound onto the outer surface 222 of the wall 220. The upper and lower flanges 73 and 75, respectively, of the blotter spool 110 engage the brake pad 221 (as in FIG. 9C) so that the length  $D_5$  of the brake pad 221 extends about midway into the width of each flange, and the thickness  $D_{16}$  of the brake pad 221 is slightly less than the unwound section  $D_1$  of the spool 80 as illustrated in FIG. 8B. The brake pad 221 is made of a material, such as foam rubber, which will compress as shown in FIG. 9C while engaged with the flanges 73 and 75 of the spool 80 and which will return to the shape shown in FIG. 9B when the spool 80 passes. Furthermore, the resilient forces of the brake pad 221 are designed to be adequate to hold the spool 80 in position along the channel 203 after the web 82 of the spool 80 has been completely unwound. FIG. 9D illustrates a film cartridge 70 engaged with the brake pad 221 so that the brake pad 221 is compressed against the wall 220, thereby creating a resilient force to hold the film cartridge 70 in place. As the film cartridge 70 passes through the channel 203, the brake pad 221 resiliently regains its original shape as shown in FIG. 9B. Of course, the brake pad 221 is but one embodiment of any means for holding a spool or cartridge at a fixed position along the channel 203.

The spindle retraction solenoid 268 is activated, causing the spindle head 278 to withdraw from engagement with the tangs 74 of the core 72 of the blotter spool 110. The spindle head 278 is drawn into the bore 282 and the brake pad 221 secures the blotter spool 110 at point C in the channel 203. The spread roll solenoid 264 is activated, causing the spreading roller 210 to disengage from the wall 220. Then, the turntable 202 is rotated clockwise to move the spool retrieval mechanism 216 along the channel 203 and into alignment with the film cartridge 70 on the spool caddy 1 as shown in FIG. 1E. The turntable 202 is momentarily stopped and the screw drive motor 262 is activated in the forward direction to extend the front support block 252 until it is positioned directly above the film cartridge 70. Once the front support block 252 is properly positioned, the screw drive motor 262 is deactivated. The spindle retraction solenoid 268 is then deactivated, causing the spindle head 278 to drop into engagement with the tangs 74 of the film cartridge 70 as previously described. After the spindle head 278 engages the tangs 74, the screw drive motor 262 is activated in the reverse direction until the front support block 252 is adjacent to the rear support block 258 and the film cartridge 70 is positioned in the channel 203. Then, the turntable 202 is rotated counterclockwise until the film 71 is completely unwound so that an emulsion side faces away from the wall 220. It is now desirable to park the film cartridge 70 along the channel 203 so that the spool retrieval mechanism 216 can retrieve other spools from the spool caddy 1.

The spindle retraction solenoid 268 is activated, causing the spindle head 278 to withdraw from engagement with the tangs 74 of the core 72 of the film cartridge 70. The spindle head 278 is drawn into the spindle bore 282 and the brake pad 221 secures the film cartridge 70 adjacent to the blotter spool 110. Then, the turntable 202 is rotated clockwise to move the spool retrieval mechanism 216 into alignment with the developer spool 80 on the spool caddy 1 as shown in FIG. 1F. At this point in time, the turntable 202 is momen-

tarily halted and the screw drive motor 262 is activated in the forward direction to extend the front support block 252 of the spool retrieval mechanism 216 until it is positioned above the core 72 of the developer spool 80. Then, the screw drive motor 262 is deactivated and the spindle retraction solenoid 268 is deactivated so that the head 278 of the spindle 276 drops into engagement with the tangs 74 of the developer spool 80. After the spindle head 278 engages the tangs 74, the screw drive motor 262 is activated in the reverse direction until the front support block 252 is adjacent to the rear support block 258 and the developer spool 80 is positioned in the channel 203. The spread roll solenoid 264 is deactivated, causing the spreading roller 210 to engage with the external side 222 of the wall 220 as previously discussed. Then, the turntable 202 is rotated counterclockwise so that developer chemical-laden absorbent layer of the developer element 82 is joined with the emulsion side of the film 71 along the external surface 222 of the wall 220. The engagement of the spreading roller 210 during unwinding results in an even spreading of chemicals imbibed within the developer element 82.

Thus, the photographic processing elements are initially brought into contact with the exposed photosensitive film with the application of force to generate pressure. Although the application of pressure can be carried out in accordance with the invention by any of various means, it is preferred to utilize a roller for the purpose, as illustrated. The roller material, the roller dimensions, the pressure which is applied, etc. can vary for any particular photosensitive film which is being processed and the particular apparatus and photoprocessing elements which are used to carry out photographic processing. Those skilled in the art will understand that where pressure is applied by means of a roller, as illustrated, for a given pressure the force needed is a function of the roller hardness, the gel strength of the absorbent layer and the carrier layer stiffness. In the preferred embodiment illustrated wherein a standard exposed 35 mm color negative film is being photographically processed it has been found that a roller having a face width of about 1.5 inches, an overall diameter of about 0.375 inch with an elastomeric outer layer such as of a polyurethane having a thickness of about 0.1 inch and a durometer hardness of about 40 (Shore-A) provides satisfactory results. Typically, a suitable applied force is in the range of from about 2 to about 10 pounds per linear inch (pli). A preferred range is from about 3 to about 6 pli and it is particularly preferred to apply a force of about 3.25 pli.

It should be noted here that the force applied during the additional application(s) of pressure may be the same as or different than that applied initially when the film and the processing element are brought into contact with each other. Also, the force applied during each additional application of pressure may be the same as or different than each other. Typically, for development of a 35 mm color negative film as illustrated, the film and the developer element 82 are allowed to remain in contact with one another for about five minutes.

The surface of spread roller 210 may be smooth as illustrated or it may be textured or embossed. Further, although the application of pressure has been illustrated with a single spread roller 210, one or more additional pressure-applying rollers can be employed. In another embodiment, the spread roller 210 can be heated, preferably to a temperature above the desired processing temperature for the processing method, to assist in bringing and maintaining the film and the processing elements to the desired processing temperature.

After the developer spool **80** comes into contact with the film cartridge **70**, the spool **80** will remain in that position for a preset developing dwell time during which the developing chemicals imbibed within the absorbent layer of the developer element **82** interact with the emulsion side of the film **71** to develop latent images. The spool retrieval mechanism **216** can be moved along the spiral wall **220**, if the spindle **276** is retracted, with the spreading roller **210** engaged throughout the developing dwell time in order to carry out the desired number of additional applications of pressure to the back of the carrier layer of the developer element **82** during the dwell time, i.e., the time period during which the developer element remains in contact with the photosensitive film. For a typical 35 mm color negative film which is processed with the standard C-41 processing, the dwell time of the developer processing element **82** is on the order of about five minutes. For the apparatus shown, a preferred number of pressure applications during the developer element dwell time is from 2 to about 10. A particularly preferred number of pressure applications is from 6 to 9.

Although the spreading roller **210** can be moved in either direction along the wall **220**, the preferred movement is unidirectional beginning at the center of the spiral wall **220**. While the spool retrieval mechanism **216** is moving back and forth along the wall **220** to allow spreading of the developer chemicals by the spreading roller **210**, the brake pad **221** secures the developer spool **80** in the channel **203** in the manner previously described.

Once the developing dwell time has expired, the spool retrieval mechanism **216** is repositioned above the developer spool **80** and the spindle retraction solenoid **268** is deactivated so that the head **278** of the spindle **276** drops into engagement with the tangs **74** of the developer spool **80**. The spread roll solenoid **264** is activated so that the spreading roller **210** is disengaged from the developer element **82**. Then, the turntable **202** is rotated clockwise with the spool rewind motor **270** simultaneously activated, causing the developer element **82** to rewind onto the developer spool **80** through the cooperative rotation of the spindle **276** and the turntable **202**. When the developer element **82** is rewound to the point where the developer spool **80** is positioned adjacent to its original position in the spool caddy **1**, the turntable **202** is deactivated. The screw drive motor **262** is activated in the forward direction to extend the front support block **252** until the developer spool **80** is again positioned in its original position in the spool caddy **1**. Then, the spool rewind motor **270** is deactivated. The screw drive motor **262** is then deactivated and the spindle retraction solenoid **268** is activated so that the head **278** of the spindle **276** is removed from engagement with the tangs **74** of the developer spool **80** and raised into the spindle bore **282**. The screw drive motor **262** is then activated in the reverse direction, causing the front support block **252** to retract to the position adjacent to the rear support block **258**. The screw drive motor **262** is then deactivated.

The turntable **202** is rotated clockwise until the spool retrieval mechanism **262** is aligned with the blix spool **90** as shown in FIG. 1G. The turntable **202** is momentarily halted and the screw drive motor **262** is again activated in the forward direction to extend the front support block **252** until it is positioned above the core **72** of the blix spool **90**. The screw drive motor **262** is stopped and the spindle retraction solenoid **268** is deactivated so that the head **278** of the spindle **276** drops into engagement with the tangs **74** of the blix spool **90**. After the spindle head **278** engages the tangs **74**, the screw drive motor **262** is activated in the reverse direction until the front support block **252** is adjacent to the

rear support block **258** and the blix spool **90** is positioned in the channel **203**. The spread roll solenoid **264** is deactivated, causing the spreading roller **210** to engage with the external side **222** of the wall **220**. Then, the turntable **202** is rotated counterclockwise until the blix spool **90** bumps into the film cartridge **70** along the channel **203** with the blix element **92** completely unwound. The unwound blix element **92** is brought into contact with the emulsion side of the film **71** so that the chemicals imbibed within the absorbent layer of the blix element **92** will bleach and fix the film **71**. Throughout a preset blix dwell time, the spool retrieval mechanism **216** with the spreading roller **210** engaged may be moved back and forth along the wall **220** with the spindle **276** retracted, as previously described, this time to evenly spread the bleaching and fixing chemicals imbibed within the absorbent layer of the blix element **92**. A typical dwell time for the blix element **92** for the illustrative film developing process is on the order of 3 minutes. It is preferred to carry out from 2 to about 5 pressure applications during this time period, and it is particularly preferred to carry out 3 or 4 pressure applications. Typically, the absorbing layer of a bleaching element contains from about 1000 to about 1200 mg/ft<sup>2</sup> (10,764–12,917 mg/m<sup>2</sup>) of active bleaching agent and that of a fixing element from about 1000 to about 1800 mg/ft<sup>2</sup> (10,764–19,375 mg/m<sup>2</sup>) of active fixing agent. The absorbent layer of a blix element, of course, contains both the active bleaching and fixing agents.

When the blix dwell time expires, the spool retrieval mechanism **216** moves back through the channel **203** to a position directly above the blix spool **90**. The above procedures are repeated for returning the blix spool **90** to the spool caddy **1**, then retrieving and unwinding a washing and stabilizing element **102** from the washing and stabilizing spool **100** on the spool caddy **1**. As is the case with the developer and blix processing elements, the absorbent layer of the unwound washing and stabilizing element **102** is brought into contact with the emulsion side of the film **71** until the spool **100** bumps into the film cartridge **70** in the channel **203**. During a washing and stabilizing dwell time, the spool retrieval mechanism **216** with the spreading roller **210** engaged and the spindle **276** retracted is moved back and forth through the channel **203**, as previously described, to spread evenly the washing and stabilizing chemicals imbibed within the absorbent layer of the washing and stabilizing element **102**. After the washing and stabilizing dwell time, the spool retrieval mechanism **216** is moved directly above the washing and stabilizing spool **100**, the web **102** is rewound, and the washing and stabilizing spool **100** is returned to its original position on the spool caddy **1**, as previously described. The wash element may contain water only or preferably may include stabilizing chemicals.

The spool retrieval mechanism **216** retrieves and rewinds both the film cartridge **70** and the blotter spool **110** to the spool caddy **1**. At this point in time, the processing of the film **71** within the film cartridge **70** is complete, and the system **200** shuts down. The user opens the cover **299** then removes and disposes of the spool caddy **1**, including the spent processing spools, and retains the processed roll of film exposures **71**, i.e. the negatives, stored on the film cartridge **70**.

The principles enunciated above are applicable for processing any number of film exposures along the spiral shaped wall **220**. Furthermore, the number of processing spools and corresponding processing steps, can be varied or reordered as necessary or desired.

The invention will now be described further in detail with respect to specific preferred embodiments by way of

examples, it being understood that these are intended to be illustrative only and the invention is not limited to materials, conditions, process parameters, etc. recited therein. All parts and percentages are by weight unless otherwise stated.

## EXAMPLE I

A rotary drum laboratory processor which was heated by circulating water through the internal cavity was used to carry out the photoprocessing experiments described below. During the experiments, which were carried out in a darkroom, the surface of the drum was maintained at a temperature of 103° F.±1° as measured by a thermocouple. The processor included a frame which allowed a 1.5 inch (38 mm) face width roller to be brought into contact with the rotating drum with varying force by application of appropriate weights.

The photosensitive film used in the experiments was Kodak Process C-41 Control Strips available from Eastman Kodak®. For a description of these control strips see Eastman Kodak Publication Z-131E2. The film was 35 mm color negative film which had been pre-exposed to an optical density step wedge.

The film was processed with four photographic processing elements, namely a developer element, a bleaching element, a fixing element and a wash element. Each photographic processing element comprised an approximately 4 mil (0.1 mm) thick polyester sheet carrying an absorbent layer made up of a 90/10 ratio of kappa carrageenan (GP911) and iota carrageenan (GP379), available from FMC Corporation, coated at a coverage of about 600 mg/ft<sup>2</sup> (6458 mg/m<sup>2</sup>) of carrageenan and about 18,000 mg/ft<sup>2</sup> (193,750 mg/m<sup>2</sup>) of water.

The respective processing fluids were imbibed into the respective processing elements by immersing a length of the processing element in a solution of the processing fluid for about three minutes followed by removing the element from the solution and removing excess solution from the surface of the processing element. A polyester cover sheet was placed over the absorbent layer until the element was used to prevent loss of fluid.

The developer layer composition solution used was

|                                   |          |
|-----------------------------------|----------|
| sodium carbonate                  | 14.228 g |
| sodium sulfite                    | 1.180 g  |
| sodium iodide                     | 0.003 g  |
| phenylmercaptotetrazole           | 0.014 g  |
| hydroxylamine sulfate             | 1.401 g  |
| CD-4 (phenylenediamene developer) | 3.570 g  |
| water                             | 250 ml   |

The bleach solution was Kodak Flexicolor RA Bleach Replenisher (Cat. No. 825 5549) diluted with an equal volume of water. The fixing solution was Kodak Flexicolor RA Fixer and Replenisher (Cat. No. 821 8950) diluted with an equal volume of water. The wash element was imbibed with water.

In operation, the absorbent layer of the photographic developer element was initially brought into contact with the emulsion layer of the photographic film with pressure applied by a polyurethane-covered roller having a diameter and durometer hardness as indicated in Table I. The developer element was allowed to remain in contact with the photographic film for five minutes during which time the drum was rotated at a speed to provide the indicated number of additional applications of pressure in accordance with the invention. After the photographic developer element contact

time was completed the developer element was removed and the bleach element, fixing element and wash element were placed in contact with the photographic film successively, each for three minutes, with the drum rotating to provide the indicated number of additional applications of pressure in accordance with the invention.

The processing parameters for the experiments are shown in Table I.

TABLE I

| Experiment | No. of Additional Applications of Pressure |    |    |    | Force* | Roller Durometer Hardness (Shore-A) | Roller Diameter (inch) |
|------------|--------------------------------------------|----|----|----|--------|-------------------------------------|------------------------|
|            | D                                          | B  | F  | W  |        |                                     |                        |
| Control-1  | 0                                          | 0  | 0  | 0  |        |                                     |                        |
| Control-2  | 23                                         | 14 | 14 | 14 | 0      | 40                                  | 0.25                   |
| 1          | 5                                          | 3  | 3  | 3  | 1.28   | 30                                  | 0.25                   |
| 2          | 5                                          | 3  | 3  | 3  | 1.28   | 30                                  | 0.50                   |
| 3          | 5                                          | 3  | 3  | 3  | 1.28   | 50                                  | 0.25                   |
| 4          | 5                                          | 3  | 3  | 3  | 1.28   | 50                                  | 0.50                   |
| 5          | 5                                          | 3  | 3  | 3  | 3.85   | 30                                  | 0.25                   |
| 6          | 5                                          | 3  | 3  | 3  | 3.85   | 30                                  | 0.50                   |
| 7          | 5                                          | 3  | 3  | 3  | 3.85   | 50                                  | 0.25                   |
| 8          | 5                                          | 3  | 3  | 3  | 3.85   | 50                                  | 0.50                   |
| 9          | 23                                         | 14 | 14 | 14 | 5.10   | 40                                  | 0.25                   |
| 10         | 23                                         | 14 | 14 | 14 | 2.55   | 30                                  | 0.25                   |
| 11         | 23                                         | 14 | 14 | 14 | 2.55   | 50                                  | 0.25                   |
| 12         | 23                                         | 14 | 14 | 14 | 2.55   | 40                                  | 0.25                   |
| 13         | 23                                         | 14 | 14 | 14 | 2.55   | 40                                  | 0.25                   |
| 14         | 23                                         | 14 | 14 | 14 | 2.55   | 40                                  | 0.25                   |
| 15         | 23                                         | 14 | 14 | 14 | 2.55   | 40                                  | 0.25                   |
| 16         | 23                                         | 14 | 14 | 14 | 2.55   | 40                                  | 0.25                   |
| 17         | 23                                         | 14 | 14 | 14 | 2.55   | 40                                  | 0.25                   |
| 18         | 23                                         | 14 | 14 | 14 | 2.55   | 40                                  | 0.50                   |
| 19         | 23                                         | 14 | 14 | 14 | 2.55   | 40                                  | 0.50                   |
| 20         | 23                                         | 14 | 14 | 14 | 2.55   | 40                                  | 0.50                   |
| 21         | 23                                         | 14 | 14 | 14 | 2.55   | 40                                  | 0.50                   |
| 22         | 23                                         | 14 | 14 | 14 | 2.55   | 40                                  | 0.50                   |
| 23         | 23                                         | 14 | 14 | 14 | 2.55   | 40                                  | 0.50                   |
| 24         | 46                                         | 28 | 28 | 28 | 1.28   | 30                                  | 0.25                   |
| 25         | 46                                         | 28 | 28 | 28 | 1.28   | 30                                  | 0.50                   |
| 26         | 46                                         | 28 | 28 | 28 | 1.28   | 50                                  | 0.25                   |
| 27         | 46                                         | 28 | 28 | 28 | 1.28   | 50                                  | 0.50                   |
| 28         | 46                                         | 28 | 28 | 28 | 3.84   | 30                                  | 0.25                   |
| 29         | 46                                         | 28 | 28 | 28 | 3.84   | 30                                  | 0.50                   |
| 30         | 46                                         | 28 | 28 | 28 | 3.84   | 50                                  | 0.25                   |
| 31         | 46                                         | 28 | 28 | 28 | 3.84   | 50                                  | 0.50                   |
| 32         | 69                                         | 41 | 41 | 41 | 2.55   | 40                                  | 0.25                   |

45 \*The force applied at the interface between the roller and the carrier layer of the processing element.

50 The sensitometry for each developed strip of photographic film was evaluated in accordance with the procedures described in Eastman Kodak Publication Z-131E2.

55 The uniformity of development in the high density wedge was measured by scanning the HD patch of the image with a Polaroid SprintScan® electronic scanner in conjunction with National Institute of Health Image Analysis Software, Version 1.61. The uniformity of the patch is characterized by analyzing the density distribution as represented by a histogram of the grey scale levels. The distribution of grey scale levels is characterized by a mean value as indicated by an individual peak in the histogram. The width of the distribution is characterized by a standard deviation as indicated by the width of an individual peak. The width of a single peak or the presence of multiple peaks is indicative of the uniformity of development or the number and extent of visual defects which are areas of poor or substantially no development.

60 65 The control-1 experiment where the photographic processing elements were initially brought into contact with the

photographic film with the application of pressure but where there were no additional applications of pressure during the time period when the film and processing elements were in contact with each other did not provide optimum sensitometry and the film exhibited numerous areas of poor or substantially no development. Similarly, the control-2 experiment, where the drum was rotated during the time period when the film and processing elements were in contact, but no force was applied to the roller and therefore no pressure was applied gave similar results.

The images obtained with experiments 12-23 exhibited substantially uniform development with improved sensitometry and lower defect levels when compared to the controls. The images from experiments 12-23 exhibited even lower defect levels.

#### EXAMPLE II

The method of the invention as carried out with an apparatus as illustrated in FIGS. 1A-1G. The film used was Polaroid HD 200 color negative film which was exposed to normal scenes including subjects and background areas. The spread roller was a 1.8 inch (45.7 mm) width roller having an overall diameter of 0.44 (11.2 mm) inch with a 0.1 inch (2.5 mm) thick outer polyurethane (45 durometer Shore-A hardness) layer. A force of 4 pounds was applied when the exposed film and each photoprocessing element were brought together and in each additional application of pressure.

The photoprocessing elements employed were of the type described in Example I. During the developer element dwell time seven additional applications of pressure were carried out and during each of the bleaching, fixing and washing element dwell times three additional pressure applications.

The developed film exhibited acceptable sensitometry and while there were some visual defects in the film indicating areas of poor development, the general uniformity of development for the film was acceptable.

It is to be understood that the above described embodiments are merely illustrative of the present invention and represent a limited number of the possible specific embodiments that can provide applications of the principles of the invention. Numerous and varied other arrangements may be readily devised in accordance with these principles by those skilled in the art without departing from the spirit and scope of the invention as claimed.

What is claimed is:

1. A method for forming a visible image in an exposed silver halide photosensitive film comprising the steps of:

(a) bringing an exposed silver halide photosensitive film

which is capable of forming a visible multicolor image into contact with a first photographic processing element with the application of pressure by pressure-applying means comprising a roller applying a force in the range of from about 2 to about 10 pounds per linear inch (pli), said first photographic processing element comprising a carrier layer and an absorbent layer containing silver halide developing material;

(b) maintaining said photosensitive film and said first photographic processing element in contact for a predetermined photographic development period and performing at least one additional pressure application step during said photographic development period with pressure-applying means comprising a roller applying a force in the range of from about 2 to about 10 pli;

(c) separating said first photographic processing element from said photosensitive film;

(d) bringing said photosensitive film into contact with a second photographic processing element with the application of pressure by pressure-applying means comprising a roller applying a force in the range of from about 2 to about 10 pli, said second photographic processing element comprising a carrier layer and an absorbent layer containing silver halide processing material;

(e) maintaining said photosensitive film and said second photographic processing element in contact for a predetermined photographic processing period and performing at least one additional pressure application step during said photographic processing period with pressure-applying means comprising a roller applying a force in the range of from about 2 to about 10 pli; and

(f) separating said second photographic processing element from said film whereby a visible image is formed in said silver halide photosensitive film.

2. The method as defined in claim 1 wherein said exposed photosensitive film includes at least three silver halide emulsions sensitized to different regions of the spectrum.

3. The method as defined in claim 2 wherein said photosensitive film is 35 mm multicolor negative film.

4. The method as defined in claim 1 wherein the absorbent layers of said first and second photographic processing elements comprise carrageenan.

5. The method as defined in claim 4 wherein the absorbent layers of said first and second photographic processing elements comprise a mixture of iota-carrageenan and kappa-carrageenan.

6. The method as defined in claim 1 wherein the force applied in at least one of steps (a), (b), (d) and (e) is in the range of from about 3 to about 6 pli.

7. The method as defined in claim 6 wherein the surface of at least one roller recited in steps (a), (b), (d) and (e) has a durometer hardness (Shore-A) of from about 40 to about 50.

8. The method as defined in claim 1 wherein from two to twelve additional applications of pressure are performed when each of said first and second photographic processing elements are in contact with said photosensitive film.

9. The method as defined in claim 1 wherein said second photographic processing element is a silver halide bleaching element including silver halide bleaching material and further including the steps of

(g) bringing said photosensitive film into contact with a third photographic processing element with the application of pressure by pressure-applying means comprising a roller applying a force in the range of from about 2 to about 10 pli, said third photographic processing element comprising a carrier layer and an absorbent layer containing silver halide fixing material;

(h) maintaining said photosensitive film and said third photographic processing element in contact for a predetermined photographic fixing period and performing at least one additional pressure application step during said fixing period with pressure-applying means comprising a roller applying a force in the range of from about 2 to about 10 pli;

(i) separating said third photographic processing element from said film;

(j) bringing said photosensitive film into contact with a fourth photographic processing element with the application of pressure by pressure-applying means comprising a roller applying a force in the range of from about 2 to about 10 pli, said fourth photographic

**23**

- processing element comprising a carrier layer and an absorbent layer containing a washing solution;
- (k) maintaining said photosensitive film and said fourth photographic processing element in contact for a pre-determined photographic washing period and performing at least one additional pressure application step during said washing period with pressure-applying means comprising a roller applying a force in the range of from about 2 to about 10 pli.
- 10.** The method as defined in claim **9** wherein the force applied in at least one of steps (g), (h), (j) and (k) is in the range of from about 3 to about 6 pli.
- 11.** The method as defined in claim **10** wherein from two to about twelve additional applications of pressure are performed when each of said first, second, third and fourth photographic processing elements are in contact with said photosensitive film.
- 12.** The method as defined in claim **11** wherein from three to nine additional applications of pressure are performed when each of said first, second, third and fourth photographic processing elements are in contact with said photosensitive film.

**24**

- 13.** The method as defined in claim **11** wherein the surface of at least one roller recited in steps (g), (h), (j) and (k) has a durometer hardness (Shore-A) of from about 40 to about 50.
- 14.** The method as defined in claim **13** wherein said photosensitive film is 35 mm multicolor negative film having at least three silver halide emulsions sensitized to different regions of the spectrum.
- 15.** The method as defined in claim **14** wherein the absorbent layers of said first, second, third and fourth photographic processing element comprise carrageenan.
- 16.** The method as defined in claim **15** wherein the absorbent layers of said first, second, third and fourth photographic processing elements comprise iota-carrageenan and kappa-carrageenan.
- 17.** The method as defined in claim **16** wherein the absorbent layers of said first, second, third and fourth absorbent layers comprise about ten percent by weight iota-carrageenan and about ninety percent by weight kappa-carrageenan.

\* \* \* \* \*